

## UNITED STATES PATENT OFFICE.

GEORGE A. RICHTER AND MILTON O. SCHUR, OF BERLIN, NEW HAMPSHIRE, ASSIGNEES TO BROWN COMPANY, OF BERLIN, NEW HAMPSHIRE, A CORPORATION OF MAINE.

## PROCESS FOR THE MANUFACTURE OF HIGH ALPHA-CELLULOSE FIBER.

No Drawing.

Application filed April 9, 1925. Serial No. 21,962.

This invention relates to the preparation of high alpha-cellulose fiber. High alpha-cellulose fiber may be produced by cooking unbleached pulp with an alkaline cooking liquor,—a caustic soda solution being especially adapted for this purpose,—and then bleaching the cooked product. This cooking may take place in digesters at any suitable temperature and pressure, although in general it has been found more economical and expedient to cook in open tanks under atmospheric pressure. The alkali in solution reacts with and dissolves the lignin and the less resistant beta and gamma celluloses of the pulp so that when the liquor is drawn off after the necessary period of digestion, the resultant product after bleaching is very white and contains about 94% alpha-cellulose fiber. High alpha-cellulose may be employed as a substitute for cotton fiber in paper-making, in the preparation of the cellulose esters, the cellulose ethers, and other compounds which require the use of substantially pure cellulose. A drawback to the use of caustic soda as the alkaline digesting-agent, however, is that it renders the process expensive. The object of this invention is to provide a more economical method for the preparation of a high alpha-cellulose fiber, yielding a product which shall possess the same characteristics as those obtained by the use of caustic soda.

Briefly, this object is attained by treating the unbleached pulp with an oxidizing agent and then cooking the treated pulp in a caustic lime solution. Other advantages are obtained by this invention, which will be subsequently pointed out.

The use of lime in cooking-liquors is old, of course, but the characteristics required of a high alpha-cellulose pulp are not realized in the product obtained from an ordinary lime treatment of the usual cellulosic materials, and so far as we know, the treatment of pulp with lime in the manner employed by us is new.

If a milk of lime cooking liquor were substituted for a caustic soda solution under the same time, pressure, and temperature conditions as in the treatment of unbleached pulp for the preparation of a high alpha-cellulose

fiber, the product obtained thereby would be much more difficult to bleach without excessive quantities of bleaching agent. This is perhaps due to the fact that slaked lime, which is a weak base and only slightly soluble in water in comparison with caustic soda, imparts a much lower alkalinity to water; consequently, such a suspension as milk of lime reacts more slowly with the lignin and other coloring matters of the unbleached pulp and in a given period of time will not have effected as complete a purification as would caustic soda. Moreover, some of the coloring matter present in the pulp may react with the lime, forming insoluble calcium compounds which are precipitated on and retained by the fiber. Hence the lignin and other coloring matter present in the pulp are, in accordance with our process, subjected to a preliminary treatment that renders these undesirable substances more easily and more completely removable by the milk of lime cooking liquor, so that fiber of pure whiteness may subsequently be obtained with a small quantity of bleach. Without such preliminary conditioning of the fiber, inasmuch as the coloring substances are not sufficiently removed by the lime digestion, in order to produce a product of the desired color it would otherwise be necessary that excessive bleach be used in the bleaching operation, with the result that the alpha-cellulose content of the pulp would suffer a material decrease owing to the partial conversion of the cellulose into oxy-cellulose, and the fiber strength would be materially affected by the excess bleach.

The extent of reaction between the relatively weak alkali and the coloring substances of the unbleached fiber may be increased by the use of a high temperature and pressure in the digestion, but this would complicate the process and call for the use of comparatively intricate apparatus, and might prove to be as expensive as a direct caustic soda treatment, if not even more expensive.

It has been found that the necessity for the use of excessive bleach may be avoided by treatment of the fiber before the lime digestion with a small quantity of oxidiz-

ing agent,—preferably chlorine. This preliminary treatment is in no sense a bleaching process, for the pulp is not at all whitened thereby; as a matter of fact, the 5 partially oxidized impurities usually impart a reddish color to the fiber. The unbleached sulphite pulp, for instance, is treated with a chlorine solution containing about 0.3% to 1.5% chlorine based on the weight of 10 fiber. The chlorine reacts with and forms compounds with a portion of the lignin and other coloring matters, rendering these more susceptible to the action of the lime cooking liquor. It is important that only a small 15 quantity of oxidizing agent be used in the preliminary treatment, for if the pulp is sensibly bleached by the oxidizing agent, the alpha-cellulose content of the final product will be low and the pulp not so well 20 suited as a substitute for cotton fiber in papermaking or for conversion into cellulose esters. The reaction with a small quantity of oxidizing agent, as for example, chlorine, is a selective one,—the more resistant 25 alpha-cellulose apparently being unaffected,—and is very rapid, the chlorine uniting with the coloring substances within a few minutes at room-temperature. The pre-treated pulp is then subjected to the action 30 of a lime cooking liquor and is boiled under conditions similar to those employed in the caustic soda solution process as hereinbefore described, where an open tank may be used. The beta and gamma cellulose constituents 35 and the coloring substances contained in the pulp are removed therefrom by reaction with the lime in solution, fresh lime from the milk of lime going into solution as the dissolved lime is consumed in the reaction. 40 The lime is effective in the removal of beta and gamma celluloses and also reacts with the coloring matter and reaction-products resulting from the chlorine treatment. The resulting pulp product is equal in quality to 45 that obtained by a direct caustic soda solution cook, and requires about the same small quantity of bleach to produce a very white, high-alpha cellulose stock.

Another important advantage may be obtained by using the chlorine pre-treatment process, which is that the wood chips may be slightly undercooked in the digesters, resulting in a longer fiber. The pulp thus produced would ordinarily be more difficult to bleach, owing to the fact that it contains a higher per cent of lignin; but the quantity of oxidizing agent used in the pre-treatment may be increased so as to react with the additional amount of lignin resulting from under-cooking. The pre-treated pulp is then subjected to the lime cooking-solution and upon bleaching yields a very white alpha-cellulose fiber of high tear test, folding endurance, and bursting strength.

65 Thus by the use of chlorine as a pre-

treating agent, caustic soda may be replaced by lime to afford a more economical method of producing high alpha-cellulose pulp of equally good quality and without the use of special apparatus.

70 A specific example of the foregoing process is approximately as follows: After wood chips have been digested in a suitable sulphite liquor, for example  $\text{Ca}(\text{HSO}_3)_2$  liquor, the digester contents are blown (slightly undercooked if so desired) and the sulphite pulp washed, screened and delivered to the open digesting tanks. The pulp is treated in the tanks at a stock-density of about 5% and at room-temperature with a chlorine solution containing 75 0.3% to 1.5% chlorine based on the weight of the fiber, the chlorine reacting with and being consumed by the ligneous matter in the pulp within a few minutes. The pulp is now washed clear of reaction products, and is squeezed to a stock-density of, say, 80 16%, then is transferred to the cooking tanks, and milk of lime added until a 10% pulp suspension is obtained, there being present about 6% to 9% reactive calcium oxide, based upon the bone-dry fiber weight. The suspension is brought to about 200° to 212° F. by blowing live steam into the 85 open tanks, and is thoroughly agitated at this temperature from five to eight hours, depending upon the characteristics of the particular sulphite pulp undergoing digestion. The less resistant beta and gamma 90 celluloses and the reactive ligneous and other coloring matter react with and are effectively removed from the pulp by the lime. After the digestion, the stock is washed clear of the reaction products in 95 the usual manner. The stock leaving the cooking tanks has approximately the following characteristics:

Alpha cellulose----- 94+%  
Fiber length----- 0.9-1.1 mm. 110  
Copper number----- 1.4-2.0.

115 The usual amount of bleach in the subsequent bleaching operation gives an alpha-cellulose fiber of high whiteness, 95 to 100 on our color-scale; the whiteness of the pulp may be increased to 100 to 110 on the same scale by a super-bleaching operation, in a chlorine solution, without loss in alpha-cellulose content.

120 While the process herein described may be practiced in the treatment of unbleached pulp produced by either an alkaline or an acid digestion, it may be employed to great advantage in the treatment of unbleached sulphite pulp to produce a high yield of fiber characterized by a very high percentage of alpha or resistant cellulose, and by a pure white color, as indicated by the specific example herein given.

125 We do not herein claim the subject matter

disclosed in our companion application, Serial No. 21,963, filed concurrently herewith, but what we claim is:

1. The process of producing high alpha-cellulose fiber from unbleached pulp, which comprises pretreating such pulp with an oxidizing liquor and then cooking such pulp in lime cooking liquor.
2. The process of producing high alpha-cellulose fiber from sulphite pulp, which comprises treating said pulp with a chlorine solution to remove or render more reactive a part of the lignin and other coloring matter, and cooking said pulp in a lime cooking liquor to remove beta and gamma celluloses and more ligneous matter therefrom.
3. The process of producing a high alpha-cellulose fiber from sulphite pulp, which comprises treating said pulp with a chlorine solution containing chlorine equal to 0.3% to 1.5% of the weight of the pulp to remove or render more reactive part of the lignin, and cooking said pulp in a lime cooking liquor to remove beta and gamma celluloses and more lignin therefrom.
4. The process of producing a high alpha-cellulose fiber from sulphite pulp, which comprises slightly undercooking chips in a sul-

phite cooking liquor, treating the pulp obtained from said sulphite digestion with a chlorine solution to remove or render more reactive part of the lignin, and cooking said pulp in a lime cooking liquor to remove the less stable beta and gamma celluloses and more lignin therefrom.

35  
5. The process of producing high alpha-cellulose fiber from sulphite pulp, which comprises treating said pulp with a chlorine solution to remove or render more reactive part of the lignin, cooking said pulp in a lime cooking liquor to remove the unstable celluloses and more ligneous matter therefrom, and bleaching the cooked pulp.

6. The process of producing a super-bleached high alpha-cellulose fiber, which comprises subjecting unbleached sulphite pulp to a preliminary oxidizing reaction, cooking with milk of lime, separating the pulp from soluble reaction products, bleaching it with calcium hydrochlorite solution and superbleaching it with a chlorine solution.

45  
In testimony whereof we have affixed our signatures.

GEORGE A. RICHTER.  
MILTON O. SCHUR.